

## UNITED STATES PATENT OFFICE.

MICHAEL F. COUGHLIN, OF STOUGHTON, MASSACHUSETTS.

## ROAD BINDER.

No Drawing.

Application filed February 24, 1922. Serial No. 539,032.

My invention has for its object an improvement in road binders composed essentially of bitumen, such as asphalt, coal tar or wax tailings. The particular object of 5 the invention is to provide a bituminous road binder which can be used cold, especially for patching road surfaces which have already been laid. It also has for its object to produce a bituminous substance dilutable 10 with water which will be capable of use as a road binder. Another and important object of my invention is to improve the binding qualities of bituminous substances such as asphalt, coal tar and wax tailings.

15 In practising my invention, I use as one element, a bitumen which is preferably but not necessarily rendered basic by the addition, if necessary, of an alkali. Coal tar may be used for this purpose and does not 20 require the addition of any alkaline substance. If liquid asphalt is used, this being acid in its natural state, I add caustic soda, calcium hydroxide or ammonia in the proportion of from  $2\frac{1}{2}$  to 5 per cent. Wax 25 tailings may be used in place of asphalt or coal tar but requires to be neutralized by the use of alkali. It will be understood of course that mixtures of various bitumens may be employed, sufficient alkali being employed to render the whole somewhat alkaline in reaction.

The bitumen, after being rendered alkaline if necessary, is mixed with a solution which is made as follows:—I take sulphite liquor of approximately  $30^{\circ}$  Baumé or a liquid made by dissolving eight (8) pounds of sulphite powder in one (1) gallon of water which gives a practically equivalent solution, and to this I add an organic acid 40 as, for instance, lactic or acetic acid, using from four (4) to eight (8) ounces of acid for each gallon of sulphite liquor. In the case of either acid, the strength is  $44^{\circ}$  Baumé.

45 The alkaline bitumen is then mixed with the sulphite liquor and acid at the ratio of five (5) parts of bitumen to one (1) of sulphite liquor and the whole thoroughly stirred to render it homogeneous.

The acid employed has the effect of reducing the viscosity of the final product, whether tar, asphalt or wax tailings be used as a base, so that it distributes itself through the gravel, stone or sand with which it is used, more readily and permeates much 55 more quickly than the ordinary bitumens alone. I also find that it affords more bond and, when incorporated with aggregates, sets more firmly.

The sulphite liquor increases the bond 60 and, being extremely hygroscopic, prevents the volatilization of the bitumen, thus acting as a preservative, greatly increasing the life of the bitumen. The acetate of lime or lactic tannate, which are believed to be 65 formed, also prevent the oil in the tar or asphalt from being volatilized and in some way cause the sulphite liquor to amalgamate with the bitumen.

I find that when mingled with a proper 70 proportion of suitable aggregates such as fine gravel, sand or broken stone, the composition may be laid cold, and when so laid, will set satisfactorily and have excellent wearing qualities due chiefly, I believe, to 75 the fact that the oils contained in the bitumen do not volatilize readily owing to the presence of the reaction products of the acids employed. Organic acid as used in the appended claims includes any capable of 80 performing those functions outlined to provide a satisfactory final product of the type described.

What I claim is—

1. The road binder which comprises a 85 basic bituminous substance, sulphite liquor, and lactic acid.
2. The road binder which comprises five parts of (a) asphalt and lime  $2\frac{1}{2}$  to 5 per cent of the asphalt and (b) one part of 90 sulphite liquor of about  $30^{\circ}$  Baumé to which has been added lactic acid in the proportion of four to eight ounces of acid to each gallon of the sulphite liquor.

In testimony whereof I affix my signature.

MICHAEL F. COUGHLIN.